



US005885302A

# United States Patent [19]

**Leuck****[11] Patent Number: 5,885,302****[45] Date of Patent: Mar. 23, 1999****[54] LEATHER TANNING PROCESS****[75] Inventor:** **Carlos Alfredo Leuck**, Rio Grande do Sul, Brazil**[73] Assignee:** **Seta S.A.—Extrativa Tanino de Acacia**, Estancia Velha, Brazil**[21] Appl. No.:** **902,594****[22] Filed:** **Jul. 30, 1997****[30] Foreign Application Priority Data**

Jul. 31, 1996 [BR] Brazil ..... 9603419-0

**[51] Int. Cl.<sup>6</sup>** ..... **C14C 3/06**; C14C 3/10; C14C 3/28**[52] U.S. Cl.** ..... **8/94.19 R**; 8/94.18; 8/94.21; 8/94.33; 8/94.26; 8/94.27; 8/94.32**[58] Field of Search** ..... 8/94.18, 94.21, 8/94.33, 94.26, 94.27, 94.32, 94.19 R**[56] References Cited****U.S. PATENT DOCUMENTS**1,659,520 2/1928 Dodge ..... 8/94.18  
2,880,053 3/1959 Fein et al. ..... 8/94.33  
3,346,324 10/1967 Fein et al. ..... 8/94.33

4,978,361 12/1990 Fuchs et al. ..... 8/94.18

**OTHER PUBLICATIONS**

T.C. Thorstensen, Practical Leather Technology, pp. 284 and 288 (month unknown), 1976.

*Primary Examiner*—Alan Diamond  
*Attorney, Agent, or Firm*—Gottlieb, Rackman & Reisman, P.C.**[57] ABSTRACT**

The present invention refers to a new process meant for chrome and/or vegetable leather tanning. The process proposed by the invention comprises the steps of bating or purging, conditioning, and chrome and/or vegetable tannage. The conditioning step uses hydroxy-butanaldehyde which reacts by blocking the amines of the collagen and releasing carboxylic acids. This reaction reduces the isoelectric point to 4.0–4.5, making the hide receptive or susceptible to effective chrome tannage by linking the carboxylic acids, or to tannin, by linking through hydrogen bridges. Hydroxybutanaldehyde is used in the conditioning step in a proportion of 2.5–3.0% as compared to the weight of the delimed hide, in a concentration of 40±2%, with a pH of 4.2–4.4, and with the reaction time being from 3 to 4 hours.

**7 Claims, No Drawings**

## LEATHER TANNING PROCESS

The present invention refers to a new process for chrome (color) and/or vegetable leather tanning.

## BACKGROUND OF THE INVENTION

The conventional process for leather tanning comprise the following operations: bathing, pickling, pre-tanning and tanning.

The bathing (purging or cleaning) of leather hides consists of deliming (removal of lime) and then bathing the hides with enzymes. The second step is the pickling operation, where the bated hide is treated with sulfuric acid and sodium chloride in order to avoid, eliminate or reduce hide deterioration. Afterwards, the pre-tanning step is executed with chrome (chromic acid) or glutaraldehyde; this is the process that gives the hide its pretanning characteristics, allowing some operations, such as splitting, and afterwards, shawing the leather. This phase results in less steps with the use of a smaller quantity of chemicals. Finally the tanning of the hide is performed with chrome (chromic acid) and/or tannins, in accordance with the specifications to be reached.

## SUMMARY OF THE INVENTION

The object of the present invention is an innovative tanning process which, through the addition of a specific product, hydroxy-butanaldehyde, to the bated or purged hide or skin, results in the conditioning of the hide or skin and, later on, chrome and/or vegetable tanning thereof. This process results in the shifting of the isoelectric point that, as the reaction time passes, varies from 3.0–3.5 to 4.0–4.5, with the pH in the same range. The process proposed by the invention allows a chrome tanning, favoring its penetration as the penetration pH range is wide, varying from 4.0 to 6.0 and the optimum point between 4.0 and 6.0 matches with the one of the process of the invention.

Advantages of the present invention over conventional tanning processes are:

- a. it is autobasifying, the addition of alkalis not being necessary;
- b. elimination of the pickle and pre-tanning phases with the subsequent removal of sulfuric acid and sodium chloride, but creating a conditioning phase;
- c. removal of sodium formate and of sodium bicarbonate used in the post-pickle treatment;
- d. simplification of the effluents treatment due to the reduction of the chrome quantity and the elimination of sodium chloride (main pollution sources of the effluents);
- e. reduction of the total tanning time, from 24–36 hours to 12–14 hours.

## DETAILED DESCRIPTION

The tanning process of the present invention comprises the steps of bathing (purging or cleaning), conditioning with hydroxy-butanaldehyde, and chrome and/or vegetable tanning. The bathing of the hide is performed in accordance with conventional tanning processes. The hydroxy-butanaldehyde is used to condition the bated hide, allowing subsequent tanning and retanning treatments, whenever it is the case. Conditioning comprises the change of the isoelectric point

of the bated hide. This is due to the hydroxy-butanaldehyde reaction with the amine. The hydroxy-butanaldehyde blocks the amines of the collagen (proteins found in greatest number in the hide), releasing the carboxyls. This, in turn,

5 reduces the isoelectric point, making the hide receptive and otherwise susceptible to effective chrome tanning (linking the carboxyls), or vegetable tanning (linking through hydrogen bridges). The percentage of hydroxy-butanaldehyde used for conditioning varies from 2.5 to 3.0% as compared to the 10 delimed hide weight, and the reaction time is approximately 3 to 4 hours. Afterwards, the tanning agent is added. In the case of chrome, the tanning time is approximately 6 to 7 hours. For vegetable tanning, the reaction time is approximately 15 12 to 14 hours.

Hydroxy-butanaldehyde is obtained from the reaction of acetic aldehyde and its structural formula is the following:



The characteristics of the product are:

mw=88.0

pH=4.2 to 4.4

concentration=40±2% of hydroxy-butanaldehyde

It will thus be seen that the objects set forth above, among those made apparent from the preceding description, are efficiently attained, and since changes may be made without departing from the spirit and scope of the invention, it is understood that the above description is merely illustrative and does not otherwise limit the scope of the invention. The 30 claims that follow define the inventive scope.

I claim:

- 35 1. A tanning process for leather comprising:  
bathing a hide or skin, the hide or skin containing collagen;  
conditioning the hide or skin by reacting hydroxybutanaldehyde with the collagen in order to block production of amines and to release carboxyls, the hide or skin having an isoelectric point that is thereby reduced to between about 4.0 and 4.5; and  
tanning the hide or skin by one of chrome and vegetable tanning.
2. The process of claim 1, wherein chrome tanning is carried out by linking chrome with the released carboxyls.
3. The process of claim 1, wherein vegetable tanning is achieved by linking the released carboxyls to the tanning compound through hydrogen bonding.
4. The process of claim 1, wherein the amount of hydroxybutanaldehyde used in the conditioning step is in the range of between 2.5 and 3.0 weight percent as compared to the overall weight of the hide or skin.
5. The process of claim 1, wherein said conditioning step has a reaction time of between about three and four hours.
6. The process of claim 1, wherein chrome tanning is carried out for a time period between about six and seven hours.
7. The process of claim 3, wherein vegetable tanning is carried out for a time period of between twelve and fourteen hours.

\* \* \* \* \*